

April 8, 1952

L. C. HENSLY  
PHOTOGRAPHIC EMULSIONS CONTAINING SYMMETRICAL  
TETRANUCLEAR DYE SALTS

2,592,515

Filed Oct. 31, 1950

2 SHEETS—SHEET 1

EMULSION CONTAINING DYE SALT OF EXAMPLE I

Fig. 1.



EMULSION CONTAINING DYE SALT OF EXAMPLE II

Fig. 2.



EMULSION CONTAINING DYE SALT OF EXAMPLE III

Fig. 3.



EMULSION CONTAINING DYE SALT OF EXAMPLE IV

Fig. 4.



INVENTOR

Lee C. Hensley

BY *Henry B. Kelley*  
*Henry B. Kelley*  
ATTORNEYS

April 8, 1952

L. C. HENSLEY  
PHOTOGRAPHIC EMULSIONS CONTAINING SYMMETRICAL  
TETRANUCLEAR DYE SALTS

2,592,515

Filed Oct. 31, 1950

2 SHEETS—SHEET 2

Fig. 5.



Fig. 6.



Fig. 7.



Fig. 8.



INVENTOR  
Lee C. Hensley

BY *Lee C. Hensley*  
*Henry B. Pelley*  
ATTORNEYS

## UNITED STATES PATENT OFFICE

2,592,515

PHOTOGRAPHIC EMULSIONS CONTAINING  
SYMMETRICAL TETRANUCLEAR DYE  
SALTSLee C. Hensley, Binghamton, N. Y., assignor to  
General Aniline & Film Corporation, New York,  
N. Y., a corporation of Delaware

Application October 31, 1950, Serial No. 193,284

6 Claims. (CL 95—7)

1

This invention relates to gelatino silver halide emulsions, and particularly to photographic emulsions sensitized by means of new symmetrical tetranuclear dye salts in which the central nucleus, 4,4'-bithiazole, is linked to two heterocyclic nitrogenous nuclei by a mono or polymethine chain.

The use of sensitizing dyes, particularly in multilayer color film, poses many problems. It is known that sensitizing dyes operate by dyeing the silver halide grain. To do this, they must be adsorbed to the silver halide. If they are displaced from the silver halide grains, they lose their effectiveness as sensitizers. It is also known that many color formers used in color photography have greater affinity for silver halides than the sensitizers, and act to displace the same from the silver halide grains. One must, therefore, select a sensitizer which will not be so displaced.

Another problem arises as regards the migration of the sensitizers from one emulsion to another. Where this ensues, color distortion is the inevitable result. Many proposals have been made dealing with the anchoring of compounds in silver halide emulsions, the most noteworthy being the use of a long alkyl chain (see Wilmanns et al. United States Patent 2,186,849).

It is, therefore, necessary, when providing sensitizers, particularly for color photography, to make certain that they have (1) the proper sensitizing power, (2) the ability to withstand displacement from silver halide grains by color formers, and (3) the ability to resist diffusion from one sensitized emulsion to another.

Efforts which satisfy the last prerequisite, unfortunately, often lead to compounds which will not meet the first two tests. Thus, it is known that the sensitizing power of cyanine dyes varies with the substituent on the cyanine N-atoms. Where this substituent is alkyl, the power decreases as the chain length increases. Hence, if a long alkyl chain be used to anchor the dye in the emulsion, we end up with a product of little or no sensitizing power. The use of other expedients to anchor the dye, on the other hand,

2

often gives products incapable of withstanding the displacement action of color formers insofar as the silver halide grains are concerned. It is thus manifest that the provision of sensitizers having the necessary prerequisite is a difficult problem, to say the least.

It is known that many cyanine dyes sensitize photographic silver halide emulsions to high red sensitivity. Most of these dyes, however, are not suitable for sensitizing silver halide emulsions containing color coupling components. This is thought to be due to a physical displacement which the sensitizing dye undergoes when color coupling components are added. That is, the sensitizer is adsorbed to the surface of the silver halide grain, and then with addition of color coupling component, is displaced therefrom.

An object of the present invention is to provide photographic silver halide emulsions with new symmetrical tetranuclear dyes containing a 4,4'-bithiazole nucleus.

A further object is to provide such dyes which are free from the disadvantages noted above.

Other objects and advantages of this invention will become apparent by reference to the following specification in which its preferred details and embodiments are described.

This invention is predicated upon the discovery that symmetrical tetranuclear dye salts, in which the central nucleus, 4,4'-bithiazole, is linked to two heterocyclic nitrogenous nuclei by a mono or polymethine chain, are not only sensitizers for orthochromatic and pancromatic film emulsions but are also compatible with color coupling components being unaffected by the presence of color coupling components and exhibiting the property of non-migration from the layer in which they are incorporated. In the latter combination, the sensitizing action of the dye salts is not impaired or diminished. An additional advantage of these dye salts is their ability to remain fixed in the layer in which they are originally deposited.

The symmetrical tetranuclear dyestuffs fulfilling the above advantages are characterized by the following general formulae:



and



## 3

wherein R is an alkyl or aralkyl group, e. g., methyl, ethyl, propyl, butyl, amyl, etc., benzyl, phenethyl and the like, R<sub>1</sub> and R<sub>2</sub> are either hydrogen or an alkyl group, e. g., methyl, ethyl, propyl, butyl, and the like, R<sub>1</sub> being only hydrogen when n equals 1, X represents an anionic acid radical, e. g., Cl, Br, I, ClO<sub>4</sub>, SO<sub>4</sub>CH<sub>3</sub>, SO<sub>4</sub>C<sub>2</sub>H<sub>5</sub>, SO<sub>3</sub>C<sub>6</sub>H<sub>4</sub>CH<sub>3</sub>, and the like, Z represents the atoms necessary to complete a 5- or 6-membered nitrogenous heterocyclic system of the type usual in cyanine dyes, such as pyridine, lepidine, quinoline, indoline, oxazole, thiazoline, thiazole, thiodiazole, pyrrolidine, selenazole, selenazoline, oxazoline, benzothiazole, benzoselenazole, benzoxazole, naphthothiazole, perinaphthiazole, naphthoselenazole, and the like, and n represents a positive integer ranging from 1 to 2.

The process of preparing the above tetranuclear cyanine dyes comprises condensing by gentle heating or boiling, or by heating as on a steam bath or under reflux conditions, one mol of a diquaternary cyclammonium salt of 2,2'-dimethyl-4,4'-bithiazole with two mols of a cyclammonium quaternary cyanine dye intermediate of the type used in the preparation of cyanine dyes. This condensation is carried out in the presence of an acid binding agent, such as nitrogenous heterocyclic base containing a small quantity of a tertiary base which may include a small quantity of acetic acid or acetic anhydride. The anions of the dye salts thus obtained are readily converted into different anions by methods well known in the art.

The diquaternary cyclammonium salts of 2,2'-dimethyl-4,4'-bithiazole utilized in the condensation reaction are characterized by the following general formula:



wherein R and X have the same values as above, and are obtained by quaternizing 2,2'-dimethyl-4,4'-bithiazole characterized by the following formula:



The 2,2'-dimethyl-4,4'-bithiazole is prepared in the following manner:

Eight and six-tenths grams (0.1 mol) of butanedione-2,3 (diacetyl) in 35 cc. of carbon disulfide were treated dropwise with stirring, with a solution of 10.6 cc. of bromine in 20 cc. of carbon disulfide at the boiling point of the carbon disulfide. The addition was completed in 3 hours. The stirring and heating were continued another 2 hours. After cooling, the carbon disulfide was decanted from the solid which had separated. The crystals were washed with petroleum ether (B. P. 60-75° C.). The melting point of the crude product was 109-111° C. After crystallizing from petroleum ether (B. P. 60-75° C.), the melting point was 117° C. and the yield of the product was 13.6 grams.

One gram of 1,4-dibromobutanedione-2,3 and 0.63 gram of thioacetamide were dissolved in 20 cc. of absolute methanol and warmed for 10 minutes on the steam bath. The mixture (a solid had separated) was poured into 100 cc. of water. The

5

aqueous mixture was made acid with diluted hydrochloric acid and filtered. Upon neutralization, a brownish solid appeared in the filtrate. This solid was filtered off and recrystallized from methanol and had a melting point of 165° C.

The quaternization of the 2,2'-dimethyl-4,4'-bithiazole is effectuated by fusion with an alkylating agent, e. g., an alkyl or aralkyl halide or by heating the base with an alkylating agent, e. g., an alkyl or aralkyl halide in a sealed tube in a water bath under increased pressure in the usual manner. The alkylating agent employed may be methyl or ethyl iodide, dimethyl sulfate, methyl p-toluenesulfonate, phenethyl iodide, and the like.

The cyclammonium salts of the type used or proposed for the production of cyanine dyes, and utilized in accordance with the present invention may be any one of those having an appropriate group in the reactive position to the nitrogen atom thereof. As examples of suitable cyclammonium quaternary cyanine dye salt intermediates having a reactive group in the 2-position to the nitrogen atom thereof so as to form a dimonomethine dye, the following may be mentioned:

25 2-methylmercapto-6-methylquinoline ethiodide  
2-methylmercapto-4-pyridine ethiodide  
2-methylmercaptothiazoline ethiodide  
2-phenylmercaptothiazoline ethiodide, and the like.

In preparing straight chain di-trimethine cyanine dye salts and branched chain di-trimethine dye salts, the following cyclammonium quaternary dye salt intermediates having a reactive group in the β-position of the side chain in the 2-position of the nitrogen atom thereof may be employed:

40 2-(β-acetanilidovinyl) thiazoline ethiodide  
2-(β-acetanilidovinyl) benzothiazole ethiodide  
2-(β-acetanilidovinyl) benzoxazole ethiodide  
2-(β-ethyl-β-methylmercapto-phenyl)-5-methoxy-benzoselenazole ethiodide  
2-(β-methylmercapto-β-methylvinyl) benzothiazole ethiodide  
45 2-(β-methylmercapto-β-propylvinyl) benzothiazole ethiodide.

In preparing straight chain or branched di-pentamethine and diheptamethine cyanine dye salts, the following cyclammonium quaternary salts having a reactive group in delta and zeta-positions of the side chain in 2-position of the nitrogen atom thereof may be employed:

55 50 2-(4-acetanilido-1,3-butadienyl) pyridine ethiodide  
2-(4-acetanilido-1,3-butadienyl) benzoxazole ethiodide  
2-(4-ethoxy-1,3-butadienyl) pyridine ethiodide  
60 2-(4-anilino-3-methyl-1,3-butadienyl) pyridine ethiodide  
2-(4-anilino-3-methyl-1,3-butadienyl)-β-naphthoxazole ethiodide  
2-(4-anilino-3-ethyl-1,3-butadienyl)-α-naphthothiazole ethiodide  
65 2-(6-anilino-1,3,5-hexatrienyl) thiazoline ethiodide  
2-(6-anilino-1,3,5-hexatrienyl)-α-naphthothiazole ethiodide  
70 2-(6-anilino-1,3,5-hexatrienyl)-β-naphthothiazole ethiodide  
2-(6-anilino-1,3,5-hexatrienyl)-α-naphthoselenazole ethiodide  
2-(6-anilino-1,3,5-hexatrienyl)-β-naphthoselenazole ethiodide

## 4

## 5

2-(6-anilino-4-methyl-1,3,5-hexatrienyl)thiazoline ethiodide  
2-(6-anilino-4-methyl-1,3,5-hexatrienyl)benzothiazole ethiodide  
2-(6-anilino-4-butyl-1,3,5-hexatrienyl)benzothiazole ethiodide.

The above cyclammonium quaternary dye salt intermediates are well known to the art and hence the methods for their preparation need



not be discussed herein. While the above dye intermediates are disclosed as being in the form of the preferred ethiodide, it is to be understood that they may also be employed in the form of other quaternary salts previously mentioned.

In the preparation of these new symmetrical tetrnuclear dyestuffs, the 2,2'-dimethyl-4,4'-bithiazole base is converted into the corresponding alkyl or aralkyl quaternary cyclammonium salt in the manner usual with the conversion of other nitrogenous heterocyclic bases to the quaternary salt form. As previously pointed out, this may be effected by fusion with alkyl or aralkyl halide or by heating the base with an alkyl or aralkyl halide in a sealed tube in a water bath under increased pressure. A molecular equivalent of the quaternary salt thus obtained is heated with two molecular equivalents of the cyclammonium cyanine dye salt intermediate in the presence of a condensing agent, such as a heterocyclic nitrogenous base or an alcohol containing a small quantity of a tertiary base at reflux temperature.

As condensing agents employed in the preparation of the new dyes of the present invention, the following may be advantageously employed: heterocyclic nitrogenous bases, such as pyridine, methylpyridine, dimethylpyridine, ethylpyridine, ethylmethylpyridine, trimethylpyridine, quinoline and the like, or an alcohol, such as methyl, ethyl, propyl, isopropyl, butyl, isobutyl, and the like, in the presence of a basic tertiary catalyst, such as trimethylamine, triethylamine, and the like.

The following examples describe in detail the methods for accomplishing the above objects, but it is to be understood that they are inserted merely for the purpose of illustration and are not to be construed as limiting the scope of the invention.

## Example I



Seven tenths gram of 2-methylmercapto-6-methylquinoline ethiodide and 0.6 gram of 2,2'-dimethyl-4,4'-bithiazole di-(ethyl p-toluenesulfonate) in 8 cc. of methanol containing 0.5 cc. of triethylamine were gently heated until methylmercaptan ceased to be evolved. After standing several hours, the solid was filtered by suction. The dye was purified by boiling with a small

## 6

amount of methanol and crystallized from pyridine.

The purified product has a melting point of 245-246° C. A methanol solution of the dye showed an absorption maximum at 497 m $\mu$ . The dye sensitized a silver bromoiodide emulsion from 450 m $\mu$  to 570 m $\mu$ , with a sensitivity maximum at 540 m $\mu$ .

## Example II



Fifty-five hundredths gram of 2,2'-dimethyl-4,4'-bithiazole di-(ethyl p-toluenesulfonate) was dissolved in 10 cc. of methanol with slight warming. To this mixture 8 drops of triethylamine were added. After 2 to 3 minutes, 1.1 grams of 2-( $\beta$ -ethyl- $\beta$ -methylmercaptovinyl)-5-methoxybenzoselenazole ethiodide were added and the mixture gently boiled for 10 minutes. After cooling the reaction mixture, 25 cc. of 10% aqueous potassium iodide solution were added with stirring. After standing a short time, the solid was filtered off and washed with ether. The crude dye was digested in 50 cc. of an equal mixture of methanol and isopropanol. After standing overnight, the dye was filtered off and recrystallized from the methanol.

The yield of the dye obtained was 0.47 gram with a melting point of 230-232° C. A methanol solution of the dye showed an absorption maximum at 571 m $\mu$ . The dye sensitized a silver bromoiodide emulsion from 500 m $\mu$  to 655 m $\mu$ , with a sensitivity maximum at 620 m $\mu$ .

## Example III



One gram of 2-( $\beta$ -acetanilidovinyl)-5,6-methylenedioxybenzothiazole ethiodide, 6 gram of 2,2'-dimethyl-4,4'-bithiazole di-(ethyl p-toluenesulfonate), 25 cc. of pyridine, and 1 cc. of triethylamine were gently boiled for 15 minutes. After cooling, two volumes of dilute aqueous potassium iodide were added. The solid was filtered off and washed with water and then ether. The product was purified by (1) digesting with isopropanol, (2) digesting with an equal mixture of methanol and isopropanol, (3) digest-

ing with methanol. The mixture was allowed to cool each time before the product was filtered off. The weight of the final product was 0.45 gram with a melting point of 249-259° C. A methanol solution of the dye showed an absorption maximum at 600 m $\mu$ . The dye sensitized a silver bromoiodide emulsion from 520 m $\mu$  to 670 m $\mu$ , with a sensitivity at 640 m $\mu$ .

## Example IV



Fifty-six hundredths gram of 2,3-dihydro-3-ethyl-5,6-methylenedioxy-2-thioacetanilidovinylbenzothiazole, 1 gram of methyl p-toluenesulfonate, and 0.3 gram of 2,2'-dimethyl-4,4'-bithiazole di-(ethyl p-toluenesulfonate) were warmed gently in a free flame with stirring for 4-5 minutes. Five cc. of methanol were added and the mixture boiled until about half of the methanol had boiled off. Twenty-five cc. of pyridine and 15 drops of triethylamine were added and the mixture boiled for 5 minutes. After cooling, 100 cc. of a 10% potassium iodide solution were added to the reaction solution with stirring. The mixture was allowed to stand 3 hours, the product filtered off and air dried. The dye was digested with 70 cc. of isopropanol. After cooling, the solid was filtered off, dissolved in 150 cc. of hot methanol, filtered while hot, and the filtrate evaporated to about 70 cc. The addition of about one-half volume of ether caused the dye to separate as a powder.

The yield of the final dye was 0.13 gram having a melting point of 267-269° C. A methanol solution of the dye showed an absorption maximum at 573 m $\mu$ . The dye sensitized a silver bromoiodide emulsion from 500 m $\mu$  to 645 m $\mu$  with a sensitivity maximum at 620 m $\mu$ .

## Example V



Five tenths gram of 2-( $\beta$ -acetanilidovinyl)-4,5-benzobenzothiazole methiodide and 0.3 gram of 2,2'-dimethyl-4,4'-bithiazole di-(ethyl p-toluenesulfonate) in 10 cc. of pyridine containing 10 drops of triethylamine were stirred at room temperature for 5 minutes and then gently boiled for 5 minutes. After cooling, the reaction mixture was diluted with 25 cc. of a 10% aqueous solution of potassium iodide. After an hour, the product was filtered off and washed with water and then ether. The product was digested for 15 minutes with 40 cc. of isopropanol. After cooling, the product was filtered off and re-digested twice with 40 cc. portions of methanol.

The yield of the purified dye was 0.3 gram with a melting point of 236-237° C. A methanol solution of the dye showed an absorption maximum at 590 m $\mu$ . The dye sensitized a silver bromoiodide emulsion from 510 m $\mu$  to 680 m $\mu$ , with a sensitivity maximum at 640 m $\mu$ .

## Example VI



Forty-five hundredths gram of 2,2'-dimethyl-4,4'-bithiazole di-(ethyl p-toluenesulfonate) and 75 grams of the dye added to a liter of emulsion.

0.8 gram of 2-( $\beta$ -acetanilidovinyl)benzothiazole in 25 cc. of n-propanol containing a few drops of triethylamine were heated, at gentle reflux, for 18 minutes. The solid that separated on cooling was washed with ether and n-propanol. It was then digested with n-propanol. After cooling, the dye was filtered and dried.

The yield of the final dye was 0.3 gram with a melting point of 230° C. A methanol solution of the dye showed an absorption maximum at 577 m $\mu$ . The dye sensitized a silver bromoiodide emulsion from 500 m $\mu$  to 650 m $\mu$ , with a sensitivity maximum at 610 m $\mu$ .

## Example VII



Eighty-seven hundredths gram of 2-( $\beta$ -acetanilidovinyl)benzoxazole ethiodide and 0.6 gram of 2,2'-dimethyl-4,4'-bithiazole di-ethiodide were dissolved in 30 cc. of methanol and warmed on a steam bath for 15 minutes in the presence of 10 drops of triethylamine. Five drops of a 40% aqueous solution of sodium perchlorate were added and the mixture warmed another 15 minutes. After cooling, the crystals were filtered off and recrystallized from methanol.

The crystallized dye has a melting point of 273-274° C. A methanol solution of the dye showed an absorption maximum at 532 m $\mu$ . The dye sensitized a silver bromoiodide emulsion from 460 m $\mu$  to 605 m $\mu$  with a sensitivity maximum at 560 m $\mu$ .

## Example VIII



One and fifteen hundredths gram of 2-( $\beta$ -acetanilidobutadienyl)benzoxazole ethiodide, 0.98 gram of 2,2'-dimethyl-4,4'-bithiazole di-(phenoxyethyl p-toluenesulfonate), and 8 drops of triethylamine were stirred for 5 minutes at room temperature in 6 cc. of pyridine. The solution was then gently boiled for 4 minutes. After cooling, the dye was precipitated by adding 2 volumes of a 20% aqueous potassium iodide solution. The product was dissolved in methanol and precipitated by the addition of a small amount of water. The dye after being crystallized twice from methanol melted at 193-195° C.

The absorption maximum in methanol is 613 m $\mu$ . The sensitization maximum in a silver iodobromide emulsion is at 665 m $\mu$  with the sensitivity range extending from 540 m $\mu$  to 700 m $\mu$ .

In the preparation of emulsions containing these tetranuclear cyanine dyes, the dye may be dissolved in methyl or ethyl alcohol and the alcoholic solution containing from 5 to 50 milligrams of the dye added to a liter of emulsion.

While in general practice, it may not be necessary to add the dye in amounts larger than those above given, generally, for satisfactory results, amounts ranging from 5 to 25 milligrams are sufficient to obtain the maximum sensitizing effect. However, I do not wish to limit my invention to the quantities just indicated as the most suitable amount will in each case be found by a few comparative experiments. The dyes may be added to the emulsion in the form of solutions. Suitable solvents, as indicated in the examples, are the alcohols, for instance, methyl or ethyl alcohol, which may be anhydrous or diluted with a small volume of water. In actual practice, the dyes are applied to the emulsion during any stage of its production. However, they are preferably added to the finished emulsion before coating.



and



The diagrammatic spectrograms constituting the accompanying drawing illustrate the regions of the spectrum to which some of the tetranuclear cyanine dyes will sensitize a gelatino silver halide emulsion containing about 4-5% of silver halide and the extent of the sensitization at various wavelengths. Figures 1 to 8 of this drawing illustrate the sensitizing properties of the dyes prepared in accordance with Examples 1 to 8, respectively.

This application is a continuation-in-part of my application Serial No. 92,584, filed May 11, 1949, now abandoned, which was a division of applica-

10  
ferred procedures, materials, and uses; it is to be understood that the new classes of tetranuclear cyanine dyes and their use as sensitizing dyes is not limited thereto and numerous variations and modifications may be made, as for example, by condensing the diquaternary ammonium salt of 2,2'-dimethyl-4,4'-bithiazole with a dialkylaminobenzene in the presence of a basic condensing agent, e. g., piperidine, di-styryl dyes are obtained. Accordingly, it is intended that the invention be defined only by the accompanying claims.

I claim:

1. A photographic gelatino silver halide emulsion which contains a dyestuff characterized by the formula selected from the class consisting of the following formulae:



35  
wherein R represents a member selected from the class consisting of alkyl and aralkyl groups, R1 and R2 represent members selected from the class consisting of hydrogen and alkyl groups, R1 being only hydrogen when n equals 1, n represents a positive integer ranging from 1 to 2, X represents an anionic radical, and Z represents the atoms necessary to complete a member of the group consisting of 5- and 6-membered nitrogenous heterocyclic ring system.

40  
2. A photographic gelatino silver halide emulsion which contains a dyestuff of the following structure:



45  
3. A photographic gelatino silver halide emulsion which contains a dyestuff of the following structure:



tion Serial No. 67, 075, filed December 23, 1948, now abandoned. The sensitizing dyestuffs per se

are claimed in application Serial No. 193,283, filed October 31, 1950.

While the present invention has been described in considerable detail with respect to certain pre-

4. A photographic gelatino silver halide emulsion which contains a dyestuff of the following structure:



11

5. A photographic gelatino silver halide emulsion which contains a dyestuff of the following structure:



5

10

12

6. A photographic gelatino silver halide emulsion which contains a dyestuff of the following structure:



LEE C. HENSLEY.

No references cited.